

SULFUR-CONTAINING LUBRICANT INHIBITED  
AGAINST STAINING

Howard M. Rue, Media, Pa., assignor to Sun Oil Company, Philadelphia, Pa., a corporation of New Jersey

No Drawing. Filed Oct. 11, 1956, Ser. No. 615,233

10 Claims. (Cl. 252—34.7)

This invention relates to sulfur-containing lubricants normally tending to stain ferrous metals, which lubricants contain a plurality of additive materials to reduce the staining tendency.

Sulfur-containing lubricants constitute a well known class of lubricants, the sulfur content providing extreme pressure properties and other beneficial properties as well known in the art. One common use of sulfur-containing lubricants is as cutting fluids of the non-emulsion type for use in metal working operations.

A difficult problem encountered in the use of sulfur-containing lubricants, particularly as cutting fluids, is the tendency of such lubricants to stain ferrous metals or other types of metals with which they come in contact in the presence of moisture. Various means have been proposed for overcoming the staining tendency, and some of these means apparently give satisfactory results when the oils are subjected to relatively mild staining tests. However, under more severe conditions tending to result in staining, measures which are satisfactory under milder conditions frequently do not provide satisfactory results.

According to the invention, a plurality of additives are employed in a sulfur-containing lubricant in order to provide a lubricating composition which is remarkably free from staining tendency even under severe testing conditions.

The additives employed in combination according to the invention are (1) a partial ester of a polyhydric alcohol, which ester has 14 to 56 carbon atoms per molecule, and (2) an acyclic polyamine having 12 to 28 carbon atoms per molecule. In one embodiment of the invention, the second additive comprises a salt of the acyclic polyamine with an organic carboxylic acid having 12 to 30 carbon atoms per molecule.

It is essential according to the invention that the specified additives be employed in combination. Neither additive alone is capable of preventing staining under severe testing conditions, whereas the combination of additives is highly effective even under severe testing conditions.

Any suitable polyhydric alcohol having two or more hydroxyl groups per molecule, can be employed in the preparation of the ester additive according to the invention. Examples of suitable ester-forming polyhydric alcohols are glycols such as ethylene glycol, propylene glycol, butylene glycol, 1,5-pentanediol, 1,6-hexanediol, diethylene glycol, triethylene glycol and higher analogs; glycerol; pentaerythritol; sorbitol; mannitol, etc. Glycerol is a preferred polyhydric alcohol for preparation of the ester additive. For further disclosure of polyhydric alcohols, reference is made to R. E. Kirk et al., "Encyclopedia of Chemical Technology," volume 1 (1947), page 308, Tables II and III, and pages 321 to 333.

The ester additive contains unesterified hydroxyl groups. Alkoxylated derivatives of the esters, prepared

by reaction of alkylene oxides with one or more of the free hydroxyl groups, can be employed if desired.

The polyhydric alcohol partial ester employed is capable of acting as a water-in-oil emulsifying agent, and accordingly has hydrophilic-lipophile balance (HLB), as defined in an article by W. C. Griffin, in "Journal of the Society of Cosmetic Chemists," volume 1, page 311 (1949), within the approximate range from 3 to 6. Examples of polyhydric alcohol partial esters which are suitable for use according to the invention are glycerol monooleate, sorbitan monostearate (Atlas Powder Company's "Span 60"), sorbitan monooleate (Atlas' "Span 80"), sorbitan sesquioleate (Atlas' "Arlacel C"), polyoxyethylene sorbitol tetraoleate having viscosity of 200-15 300 cp. at 25° C. and specific gravity of 0.92-0.98 (Atlas' "G-2854"), polyoxyethylene sorbitol pentaoleate having viscosity of 100-200 cp. at 25° C. and specific gravity of 0.92-0.98 (Atlas' "G-2855"), polyoxyethylene sorbitol cottonseed oil derivative having viscosity of 20 100-200 cp. at 25° C. and specific gravity of 0.92-0.98 (Atlas' "G-931"), etc.

It is within the ability of a person skilled in the art to obtain a desired HLB value for partial esters of a given polyhydric alcohol as disclosed previously herein, by 25 proper adjustment of the hydrophilic and lipophilic parts of the molecule. Thus, for example, the molecule may be made more hydrophilic (i.e. higher HLB) in a given instance by introducing polyoxyalkylene radicals into the molecule. Or the molecule may be made more lipophilic (i.e. lower HLB) by introducing additional long chain fatty acid radicals into the molecule or by increasing the chain length of the fatty acid radical or radicals; thus for example, sorbitan trioleate has lower HLB than sorbitan monooleate, and the latter has lower 35 HLB than sorbitan monolaurate. The number of hydroxyl groups in the polyhydric alcohol has an effect on the HLB value, free hydroxyl groups generally increasing the HLB value. By proper adjustment of these factors, a person skilled in the art can make, in addition to the specific esters mentioned above, numerous other water-in-oil emulsifying agents suitable for use according to the invention.

Any suitable organic monocarboxylic acid can be employed in the preparation of the ester additive. Thus, 45 the acid can be an aromatic, aliphatic, cycloaliphatic or heterocyclic carboxylic acid. Preferred acids are: the naturally occurring fatty acids, more preferably those having 12 to 30 carbon atoms per molecule, e.g. lauric, myristic, palmitic, oleic, stearic, erucic acids, etc.; petroleum naphthenic acids; rosin acids; and mixtures of carboxylic acids obtained by the partial oxidation in liquid phase of hydrocarbon mixtures such as petroleum fractions, as disclosed in L. W. Jones United States Patent No. 2,756,211 issued July 24, 1956, and the disclosures 55 referred to in the specification of that patent. Other types of acids can be employed to make the ester additive, e.g. benzoic acid, furoic acid, etc. However, the acids previously mentioned are preferred.

The number of carbon atoms in the acid varies according to the nature of the rest of the molecule, that number being one of a plurality of factors influencing HLB. Thus, for example, in the case of glycerol monoesters and the other esters previously specifically disclosed, the acid or acids preferably have 16 to 22 carbon atoms per 60 molecule, or an average of 16 to 22 carbon atoms per molecule. In other esters, higher or lower molecular weight acids may be required, as readily determinable by a person skilled in the art.

The polyamine additive employed according to the invention contains two or more amino groups per molecule and preferably has at least one primary amino group in the molecule, and also preferably contains at least 65

two amino groups other than a tertiary amino group. Particularly suitable polyamines are diamines having one primary amino group and one secondary amino group. The polyamine can contain any suitable number of nitrogen atoms per molecule, though generally this number does not exceed 10, and more preferably, the number of nitrogen atoms is not greater than 5. The polyamine may contain hydroxyl groups in addition to nitrogen atoms, though preferably the polyamine contains only carbon, hydrogen, and nitrogen in the molecule. Alkoxylated derivatives containing  $-(CH_2CH_2O)_nH$  groups attached to one or more nitrogen atoms, where  $n$  is an integer from 1 to 10 for example, can be employed if desired.

Where salts of the polyamines are employed, the carboxylic acid employed to make the salt can be an acid as described previously with regard to the acid employed in preparation of the ester additive. The acid employed to make the salt can be the same acid as that employed to make the ester, or it may be a different acid within the same general class. The examples of acids given previously with regard to the ester preparation constitute examples of acids which can be employed to make salts of the polyamine. Although carboxylic acid salts of the polyamines are preferred because of their generally superior corrosion inhibiting properties, the unneutralized polyamines can also be employed.

Preferred polyamine materials are the salts of an organic carboxylic acid having 12 to 30 carbon atoms per molecule and a polyamine having the formula



where  $R$  is a hydrocarbon radical containing 10 to 30 carbon atoms and  $n$  is an integer from 2 to 6. Mono- or disalts can be employed. Examples of suitable carboxylic acids are fatty acids, naphthenic acids, rosin acids, acids produced by partial oxidation in liquid phase of petroleum fractions etc. Examples of suitable  $R$  radicals are the hydrocarbon residues from such carboxylic acids. Examples of suitable polyamines are alkylene diamines such as ethylene diamine, trimethylene diamine, tetramethylene diamine, pentamethylene diamine, and hexamethylene diamine, having an  $R$  substituent on one nitrogen atom, e.g. N-decylethylene diamine, N-hexadecyl propane diamine-1,3, N-butyl tetraethylene pentamine, N-octadecyl diethylene triamine, N-dibutyl tetramethylene diamine, N-abetyl hexamethylene diamine, N-naphthyl-N'-methyl ethylene diamine, polyethoxylated derivatives of the foregoing, etc.

Although less preferred, polyamines wherein  $R$  in the formula given in the preceding paragraph is hydrogen can also be employed, e.g. 1,2-diamino dodecane, 1,12-diamino tetradecane, diamino octadecanes, polyethoxylated derivatives of the foregoing, etc.

The invention is applicable generally to sulfur-containing lubricants which tend to stain various metals upon contact therewith, for example in the use of the sulfur-containing lubricant as a cutting fluid in the working of ferrous metals. Examples of suitable sulfur-containing lubricants are fatty or petroleum oils containing dissolved elemental sulfur, fatty or petroleum oils which have been reacted at elevated temperature with a sulfurizing agent such as elemental sulfur, sulfur monochloride, etc. Various fatty oils are suitable for this purpose, e.g. lard oil, rapeseed oil, sperm oil, cottonseed oil, palm oil, etc. Other examples of sulfur-containing lubricants are fatty or petroleum oils containing various sulfur-containing additives such as xanthate esters, metal salts of reaction products of olefins and phosphorous pentasulfide, organic trisulfides, metal salts of organic-substituted phosphoric acids, e.g. zinc, dihexyl dithiosulfide, sulfurized olefins such as sulfurized terpenes, etc.

The polyamine additive employed according to the invention can be prepared in any suitable manner. As an example of a manner of preparation of a particularly

effective polyamine, the following description is given: a carboxylic acid or mixture of acids such as tallow fatty acids can be reacted with ammonia to produce ammonium soaps, which are then chemically dehydrated by known means to form nitriles, the latter then being hydrogenated to form fatty amines; the latter are reacted with acrylonitrile to form compounds having the formula



10 where  $R$  is a hydrocarbon radical of the original fatty acid,  $RCOOH$ ; the resulting compounds are hydrogenated to provide amines having the formula



15 Such amines are highly suitable for use according to the invention. In the preparation described, other carboxylic acids as previously disclosed herein can be employed instead of fatty acids. Thus, for example, naphthenic acids, rosin acids, acids obtained by partial oxidation, etc. can be employed.

20 The following examples illustrate the invention.

The following composition was prepared:

| Component | Description                                                                                                                                          | Parts by Volume |
|-----------|------------------------------------------------------------------------------------------------------------------------------------------------------|-----------------|
| A         | Petroleum lubricating oil (Neutral distillate from naphthenic base crude, about 100 SUS at 100° F.).                                                 | 40              |
| B         | Sulfochlorinated methyl esters of lard oil acids (Reaction product of esters with $S_2Cl_2$ , S content 9 Wt. percent, Cl content 9 Wt. percent).    | 10              |
| 30 C      | Sulfur-containing petroleum oil (0.9 Wt. percent of elemental S dissolved at 140-150° F. in neutral naphthenic distillate—about 150 SUS at 100° F.). | 50              |
| D         | N-tallow propylene diamine dinaphthenate.                                                                                                            | 0.5             |
| E         | Glycerol monooleate.                                                                                                                                 | 0.5             |

35 Component D was prepared by neutralizing naphthenic acids with a material known by the trademark "Duomeen T" comprising a mixture of diamines having the formula  $RNHCH_2CH_2CH_2NH_2$  where  $R$  is a hydrocarbon radical derived from tallow, the average molecular weight of the mixture of diamines being 320, the combining weight being about 400 however because of the presence of impurities. The preparation of such diamine mixtures is described in United States Patent No. 2,736,658 issued

45 February 28, 1956, to F. W. Pfohl and V. P. Gregory.

The naphthenic acids employed in the preparation of component D conformed in preparation and properties to those sold commercially under the trademark "Sunaptic Acids C." Typical properties for such acids are the following: acid number 122 mg. of KOH per gram, average molecular weight 415, average molecular formula  $C_{28}H_{49}O_2$ , average type formula  $C_nH_{2n-7}O_2$ , and distillation range 408° F. to 596° F./2 mm. Hg (0-96%). Component D was prepared by stirring together at room temperature, and thereby reacting, about 415 parts by weight of the naphthenic acids with slightly more than 400 parts by weight of Duomeen T. The resulting mixture of salts varied from one salt to the next not only in the diamine but also in the acid since the naphthenic acids used were also a mixture of acids having varying molecular weight and chemical structure.

55 The composition described above was tested for its staining characteristics: 90 cc. of the composition and 10 cc. of water were agitated together to produce a dispersion of water in the composition; 1 cc. of the dispersion was placed between two polished steel panels, and the latter were maintained in close contact with a film of the dispersion between them for 24 hours at room temperature; the panels were then separated, washed with naphtha, and observed.

60 For comparison, compositions as described above, but containing in one instance neither component D nor component E, in another instance 1 part by volume of component D in the absence of component E, and in another instance 1 part by volume of component E in the

absence of component D, were subjected to the same test. 1 part each of components D and E were also tested in another composition. The following table shows the results:

| Parts by Volume |     | Stain        |
|-----------------|-----|--------------|
| D               | E   |              |
| 0               | 0   | Heavy.       |
| 1.0             | 0   | Heavy.       |
| 0               | 1.0 | Heavy.       |
| 0.5             | 0.5 | Very slight. |
| 1.0             | 1.0 | None.        |

These results show the necessity for both components to secure the beneficial reduction in staining tendency. No significant reduction in staining is obtained with 1 part by volume of either component alone. On the other hand, a great reduction in staining is obtained with 1 part of an equal volume mixture of the two components, and complete elimination of staining in a very severe test is obtained with 2 parts of an equal volume mixture.

Generally similar results are obtained using fatty acids such as oleic acid, rosin acids, or acids obtained by partial oxidation of hydrocarbons, in place of naphthenic acids in the preparation of component D. Generally similar results are also obtained using other specific polyhydric alcohol esters within the scope of the invention, for example the specific esters disclosed previously herein, and also sorbitan monoesters of petroleum naphthenic acids having an average of 21 carbon atoms per molecule, polyoxyethylene sorbitol tetraesters of carboxylic acids produced in liquid phase partial oxidation of petroleum lubricating oil and having an average of 18 carbon atoms per molecule, glycerol monoabietate, etc. Generally similar results are also obtained using other sulfur-containing lubricants such as sulfochlorinated lard oil containing about 2 percent each of sulfur and chlorine, or the individual component C of the above-described composition, or a lubricant obtained by reacting elemental sulfur at 300° F. with a naphthenic petroleum distillate having Saybolt Universal viscosity at 100° F. of about 160 seconds for 2 hours to produce an oil containing about 2 weight percent of sulfur, etc. Generally similar results are also obtained using other polyamines or salts such as N-decyl ethylene diamine monoabietate, N-butyl tetraethylene pentamine distearate, a mixture of polyalkylene polyamines having the formula



where  $n$  is an integer varying through the range from 6 to 10, N-octadecyl diethylene triamine trilaurate, the specific polyamines disclosed previously herein, salts of those polyamines with the specific carboxylic acids disclosed previously herein, etc. The various specific materials disclosed previously can be employed in any desired combination.

The essential characteristic of the polyamine or salt additive employed according to the invention is believed to be its ability to effectively inhibit corrosion by mixtures of oil and water in the presence of inorganic acids such as the  $\text{H}_2\text{S}$  generally present in small amounts in sulfur-containing oils, and the  $\text{HCl}$  generally present in small amounts in chlorine-containing oils. This char-

acteristic is typical of the polyamines and salts within the scope of the invention as set forth previously. The essential characteristic of the ester additive is believed to be its ability to emulsify water in oil, a characteristic which is generally typical of the esters within the scope of the invention as set forth previously.

The invention claimed is:

1. A lubricating composition consisting essentially of a sulfur-containing lubricant selected from the group consisting of petroleum hydrocarbon oils and fatty oils, which lubricant contains at least 1 weight percent of sulfur and tends to stain ferrous metals upon contact therewith, 0.1 to 5 weight percent of a partial ester of a polyhydric alcohol, said ester having hydrophile-lipophile balance within the approximate range from 3 to 6 and containing 14 to 56 carbon atoms per molecule, and 0.1 to 5 weight percent of a component selected from the group consisting of an acyclic polyamine containing 12 to 28 carbon atoms per molecule and a salt of said polyamine with an organic carboxylic acid containing 12 to 30 carbon atoms per molecule.
2. The lubricating composition of claim 1 wherein said partial ester is a monoglyceride of a naturally occurring fatty acid.
3. The lubricating composition of claim 1 wherein said polyamine is an N-substituted alkylene diamine containing 2 to 6 carbon atoms in the alkylene group between the nitrogen atoms.
4. The lubricating composition of claim 1 wherein the sulfur-containing lubricant comprises a sulfochlorinated fatty oil.
5. The lubricating composition of claim 1 wherein the sulfur-containing lubricant comprises a sulfurized mineral oil.
6. The lubricating composition of claim 1 wherein the sulfur-containing lubricant contains 1 to 5 weight percent of sulfur.
7. The lubricating composition of claim 1 wherein said ester is present in an amount which is capable of incorporation in said lubricant in the absence of said polyamine.
8. The lubricating composition of claim 1 wherein said sulfur-containing lubricant comprises a naphthenic petroleum distillate.
9. The lubricating composition of claim 1 wherein said partial ester is a monoglyceride of an organic carboxylic acid containing 12 to 30 carbon atoms per molecule, and said polyamine is an N-substituted alkylene diamine containing 2 to 6 carbon atoms in the alkylene group between the nitrogen atoms, the N-substituent being a hydrocarbon radical having 12 to 30 carbon atoms.
10. The lubricating composition of claim 9 wherein said carboxylic acid is selected from the group consisting of naturally occurring fatty acids, rosin acids, petroleum naphthenic acids, and acids obtained by partial oxidation of hydrocarbon mixtures.

#### References Cited in the file of this patent

#### UNITED STATES PATENTS

- |           |              |       |               |
|-----------|--------------|-------|---------------|
| 2,564,422 | Barnum       | ----- | Aug. 14, 1951 |
| 2,626,240 | Deutser      | ----- | Jan. 20, 1953 |
| 2,696,473 | Sokol        | ----- | Dec. 7, 1954  |
| 2,736,658 | Pfohl et al. | ----- | Feb. 28, 1956 |
| 2,798,046 | Buck et al.  | ----- | July 2, 1957  |